



US006824737B2

(12) **United States Patent**  
**Koch**

(10) **Patent No.:** **US 6,824,737 B2**  
(45) **Date of Patent:** **Nov. 30, 2004**

(54) **CASTING ALLOY**

(75) Inventor: **Hubert Koch**, Rheinfelden (DE)

(73) Assignee: **Aluminium Rheinfelden GmbH**,  
Rheinfelden (DE)

(\*) Notice: Subject to any disclaimer, the term of this  
patent is extended or adjusted under 35  
U.S.C. 154(b) by 0 days.

(21) Appl. No.: **10/761,513**

(22) Filed: **Jan. 20, 2004**

(65) **Prior Publication Data**

US 2004/0170523 A1 Sep. 2, 2004

(51) **Int. Cl.**<sup>7</sup> ..... **C22C 21/04**

(52) **U.S. Cl.** ..... **420/549; 420/553**

(58) **Field of Search** ..... **420/549, 553,  
420/548**

(56) **References Cited**

U.S. PATENT DOCUMENTS

4,995,917 A 2/1991 Dagustany et al.  
6,309,481 B1 10/2001 Koch et al.

6,364,970 B1 4/2002 Hielscher et al.

FOREIGN PATENT DOCUMENTS

|    |           |        |
|----|-----------|--------|
| EP | 0 601 972 | 6/1994 |
| FR | 1.300.416 | 8/1962 |

*Primary Examiner*—Roy King

*Assistant Examiner*—Janelle Combs Morillo

(74) *Attorney, Agent, or Firm*—Bachman & LaPointe, P.C.

(57) **ABSTRACT**

An aluminium alloy suitable for diecasting of components with high elongation in the cast state comprises, as well as aluminium and unavoidable impurities, 9.0 to 11.0 w. % silicon, 0.5 to 0.9 w. % manganese, max 0.06 w. % magnesium, 0.15 w. % iron, max 0.03 w. % copper, max 0.10 w. % zinc, max 0.15 w. % titanium, 0.05 to 0.5 w. % molybdenum and 30 to 300 ppm strontium or 5 to 30 ppm sodium and/or 1 to 30 ppm calcium for permanent refinement. Optionally, the alloy also contains 0.05 to 0.3 w. % zirconium and for grain refinement gallium phosphide and/or indium phosphide in a quantity corresponding to 1 to 250 ppm phosphorus and/or titanium and boron added by way of an aluminium master alloy with 1 to 2 w. % Ti and 1 to 2 w. % B.

**9 Claims, No Drawings**

# 1

## CASTING ALLOY

The invention concerns an aluminium alloy for diecasting of components with high elongation in the cast state.

Diecasting technology has today developed so far that it is possible to produce components with high quality standards. The quality of a diecasting however depends not only on the machine setting and the process selected but to a great extent also on the chemical composition and the structure of the aluminium alloy used. The latter two parameters are known to influence the castability, the feed behaviour (G. Schindelbauer, J. Czikel "Mould filling capacity and volume deficit of conventional aluminium diecasting alloys", Gießereiforschung 42, 1990, p. 88/89), the mechanical properties and—particularly important in diecasting—the life of the casting tools (L. A. Norström, B. Klarenfjord, M. Svenson "General Aspects on Wash-out Mechanism in Aluminium Diecasting Dies" 17th International NADCA Diecasting Congress 1993, Cleveland, Ohio).

In the past little attention has been paid to the development of aluminium alloys which are particularly suited for diecasting of high quality components. Manufacturers in the car industry are now increasingly required to produce e.g. weldable components with high ductility in the diecasting process, since diecasting is the most economic production method for high quantities.

The refinement of the diecasting technology now allows the production of weldable components of high quality. This has expanded the area of application for diecastings to include chassis components.

Ductility is increasingly important, in particular in components of complex design.

In order to achieve the required mechanical properties, in particular a high elongation to fracture, the diecastings must usually be subjected to heat treatment. This heat treatment is necessary for forming the casting phase and hence achieving ductile fracture behaviour. Heat treatment usually means solution annealing at temperatures just below the solidus temperature with subsequent quenching in water or another medium to temperatures <100° C. The material treated in this way now has a low elongation limit and tensile strength. In order to raise these properties to the required value, artificial ageing is then performed. This can also be process-induced e.g. by thermal shock on painting or stress-relief annealing of a complete assembly.

As diecastings are cast close to the final dimensions, they usually have a complex geometry with thin walls. During the solution annealing, and in particular the quenching process, distortion must be expected which can require retouching e.g. by straightening the casting or, in the worst case, rejection. Solution annealing also entails additional costs, and the efficiency of this production method could be substantially increased if alloys were available which fulfilled the required properties without heat treatment.

An AlSi alloy with good mechanical values in the casting state is known from EP-A-0 687 742. Also for example EP-A-0 911 420 discloses alloys of type AlMg which in the casting state have a very high ductility, but with complex form design however tend to hot or cold cracking and are therefore unsuitable. A further disadvantage of ductile diecastings is their slow ageing in the cast state which can lead to a temporary change in mechanical properties—including a loss of expansion. This behaviour is tolerated in many applications as the property limits are not exceeded, but cannot be tolerated in some applications and can only be excluded by targeted heat treatment.

The invention is based on the object of preparing an aluminium alloy which is suitable for diecasting which is

# 2

easy to cast, has a high elongation in the cast state and after casting ages no further. In addition the alloy should be easily weldable and flangeable, able to be riveted and have good corrosion resistance.

According to the invention the object is achieved by an aluminium alloy with

8.5 to 10.5 w. % silicon

0.3 to 0.8 w. % manganese

max 0.06 w. % magnesium

max 0.15 w. % iron

max 0.03 w. % copper

max 0.10 w. % zinc

max 0.15 w. % titanium

0.05 to 0.5 w. % molybdenum

30 to 300 ppm strontium or 5 to 30 ppm sodium and/or 1 to 30 ppm calcium for permanent refinement, optionally also

0.05 to 0.3 w. % zirconium

gallium phosphide and/or indium phosphide in a quantity corresponding to 1 to 250 ppm phosphorus for grain refinement titanium and boron added by way of an aluminium master alloy with 1 to 2 w. % Ti and 1 to 2 w. % B for grain refinement, and as the remainder aluminium and unavoidable impurities.

With the alloy composition according to the invention, for diecastings in the cast state a high elongation can be achieved with good values for the yield strength and tensile strength, so that the alloy is suitable in particular for the production of safety components in car manufacture.

Surprisingly, it has been found that by the addition of molybdenum the elongation can be increased substantially without losses in the other mechanical properties. The desired effect can be achieved with the addition of 0.05 to 0.5 w. % Mo, the preferred behaviour level is 0.08 to 0.25 w. % Mo.

With the combined addition of molybdenum and 0.05 to 0.3 w. % Zr, the elongation can be improved even further. The preferred content is 0.15 to 0.02 w. % Zr.

The relatively high proportion of eutectic silicon is refined by strontium. In contrast to granular diecasting alloys with high contaminant levels, the alloy according to the invention also has advantages with regard to fatigue strength. The fracture toughness is higher because of the very low mixed crystals present and the refined eutectic. The strontium content is preferably between 50 and 150 ppm and in general should not fall below 50 ppm otherwise the casting behaviour can deteriorate. Instead of strontium, sodium and/or calcium can be added.

By restricting the magnesium content to preferably max 0.05 w. % Mg, the eutectic structure is not coarsened and the alloy has no age-hardening potential which contributes to a high elongation.

Due to the proportion of manganese, adhesion in the mould is avoided and good mould removal properties guaranteed. The manganese content gives the casting a high structural strength at high temperature so that on removal from the mould, very little or no distortion is expected.

The alloy according to the invention can be riveted in the cast state.

With stabilisation annealing for 1 to 2 hours in a temperature range of around 280 to 320° C., very high elongation values can be achieved.

The alloy according to the invention is preferably produced as a horizontal diecasting pig. Thus without costly melt cleaning, a diecasting alloy with low oxide contami-

## 3

nation can be melted: an important condition for achieving high elongation values in the diecasting.

On melting, any contamination of the melt, in particular by copper or iron, must be avoided. The permanently refined AISi alloy according to the invention is preferably cleaned by flushing gas treatment with inert gases by means of impellers.

Preferably, grain refinement is performed in the alloy according to the invention. For this gallium phosphide and/or indium phosphide can be added to the alloy in a quantity corresponding to 1 to 250 ppm, preferably 1 to 30 ppm phosphorus. Alternatively or additionally the alloy can contain titanium and boron for grain refinement, where the titanium and boron are added by way of a master alloy with 1 to 2 w. % Ti and 1 to 2 w. % B, remainder aluminium. Preferably, the aluminium master alloy contains 1.3 to 1.8 w. % Ti and 1.3 to 1.8 w. % B and has a Ti/B weight ratio of around 0.8 to 1.2. The content of the master alloy in the alloy according to the invention is preferably set at 0.05 to 0.5 w. %.

The aluminium alloy according to the invention is particularly suitable for the production of safety components in the diecasting process.

What is claimed is:

1. Aluminium alloy for diecasting of components with high elongation in the cast state with
  - 25 8.5 to 10.5 w. % silicon
  - 0.3 to 0.8 w. % manganese
  - max 0.06 w. % magnesium
  - max 0.15 w. % iron
  - max 0.03 w. % copper
  - max 0.10 w. % zinc
  - max 0.15 w. % titanium
  - 0.05 to 0.5 w. % molybdenum

## 4

30 to 300 ppm strontium or 5 to 30 ppm sodium and/or 1 to

30 ppm calcium for permanent refinement, optionally also

0.05 to 0.3 w. % zirconium

gallium phosphide and/or indium phosphide in a quantity corresponding to 1 to 250 ppm phosphorus for grain refinement

10 titanium and boron added by way of an aluminium master alloy with 1 to 2 w. % Ti and 1 to 2 w. % B for grain refinement,

15 and as the remainder aluminium and unavoidable impurities.

2. Aluminium alloy according to claim 1, characterised by 50 to 150 ppm strontium.

3. Aluminium alloy according to claim 1, characterised by max 0.05 w. % magnesium.

20 4. Aluminium alloy according to claim 1, characterised by max 0.10 to 0.20 w. % zirconium.

5. Aluminium alloy according to claim 1, characterised by 0.08 to 0.25 w. % molybdenum.

6. Aluminium alloy according to claim 1, characterised by gallium phosphide and/or indium phosphide in a quantity corresponding to 1 to 30 ppm phosphorus.

7. Aluminium alloy according to claim 1, characterised by an aluminium master alloy with 1.3 to 1.8 w. % titanium and 1.3 to 1.8 w. % boron and a titanium/boron weight ratio between 0.8 and 1.2.

30 8. Aluminium alloy according to claim 1, characterised by 0.5 to 0.5 w. % aluminium master alloy.

9. A diecast safety component in a car comprising the aluminium alloy of claim 1.

\* \* \* \* \*